

# UNITED STATES PATENT OFFICE.

JOSEPH P. BENNETT, OF DULUTH, MINNESOTA.

## PROCESS FOR IMPREGNATING MATCH-SPLINTS.

1,372,860.

Specification of Letters Patent. Patented Mar. 29, 1921.

No Drawing.

Application filed February 26, 1920. Serial No. 361,545.

To all whom it may concern:

Be it known that I, JOSEPH P. BENNETT, a citizen of the United States, residing at Duluth, in the county of St. Louis and State 5 of Minnesota, have invented new and useful Improvements in Processes for Impregnating Match-Splints, of which the following is a specification.

My invention relates to an improved process 10 for impregnating match splints for the purpose of rendering the splints nonglowing after the matches have been used.

It has become common practice to dust upon the splints, while in a match making 15 machine of the ordinary continuous type, a fine powder such as ammonium phosphate, for the purpose of preventing the dangerous after-glow when the matches are used. Means for accomplishing this purpose are

20 described in Patent No. 1,326,633, granted to me on the 30th day of December, 1919.

The object of my present invention is to increase the efficiency of the impregnating process by securing a more uniform coating 25 and deeper penetration of the fibers of the splints by the glow-deterring material.

The usual methods now in practice are dependent for their success upon the adhesion to the surface of the splint of the fine 30 dry powder which is applied thereto. I have found that the uniformity and efficiency of impregnation is much increased by my present process which consists in subjecting the match splints to a cloud of fine powder and 35 then melting and dissolving the adhering powder by the application of steam.

To this end I first pass the splints through a cloud of fine powder, such as ammonium phosphate, which may be done by the means

pointed out in my patent above mentioned, 40 and I then expose the splints so dusted to the action of steam, preferably in an enclosed receptacle, whereby the powder is melted and dissolved and the surfaces of the fibers and interstices between the same are 45 thoroughly impregnated with the chemical forming the powder, after which the splints are removed from the steam and immersed in paraffin.

The steaming of the powdered splints, in 50 conjunction with the other steps above described, results in the economical production of better and safer matches than those produced by the methods of manufacture heretofore practised.

Having described my invention, what I 55 claim as new and desire to protect by Letters Patent is:

1. The method of treating match splints which consists in first dusting the splints 60 with a glow deterring, impregnating powder, and then steaming the splints to melt and dissolve the powder in the pores and upon the surface of the splints.

2. The method of treating match splints 65 by first dusting the same with a dry, soluble powder adapted to prevent after-glow, then steaming the splints, and finally dipping the same in paraffin.

3. The method of treating match splints 70 which consists in first dusting the same with a dry soluble powder adapted to prevent after-glow and then steaming the splints to dissolve the powder thereon.

In testimony whereof I have hereunto 75 signed my name to this specification.

JOSEPH P. BENNETT.